

# UNITED STATES PATENT OFFICE.

FRANK KAVANAUGH, OF HARRISBURG, TEXAS.

## METALLIC COMPOUND.

SPECIFICATION forming part of Letters Patent No. 323,426, dated August 4, 1885.

Application filed May 13, 1884. (Specimens.)

*To all whom it may concern:*

Be it known that I, FRANK KAVANAUGH, a citizen of the United States, residing at Harrisburg, in the county of Harris and State of Texas, have invented a new and useful Metallic Compound, of which the following is a specification.

This invention has relation to a metallic compound designed to be used as a substitute for brass and bronzes, and particularly for journal-bearings of all kinds.

The proportions of the several ingredients employed in making my composition are as follows: zinc, eighty-five and three-fourths pounds; copper, nine pounds; tin, two pounds; lead, one pound; cast-iron, one pound; sal-ammoniac, eight ounces; silica, eight ounces; refined borax, four ounces. These ingredients are melted together in a furnace and cast in molds into the form desired.

The composition is a superior anti-friction substance, and is especially adapted for use for the journals of engines, passenger and freight cars, in the place of babbitted brasses and other anti-friction metal bearings and more durable than the metals referred to. The alloy resulting from this process is found by

analysis to contain, in one hundred parts, zinc, 87; lead, 1.15; tin, 1.7, copper, 9.5; iron, .3.

I am aware that alloys containing zinc, copper, tin, lead, and iron are old in the art, and I claim them only when used with the salts sal-ammoniac, silicic acid, and refined borax as fluxes, and only when compounded in the proportions specified, as I find that the resulting alloy possesses properties that render it less liable to become hot in use, and that it is much more durable than babbitted brasses and other anti-friction metal bearings.

What I claim as new, and desire to secure by Letters Patent of the United States, is—

The process of making alloys for journal-bearings which consists in melting zinc, tin, copper, lead, and cast-iron in the proportions stated, with a flux of sal-ammoniac, silica, and borax, substantially as described.

In testimony that I claim the foregoing as my own I have hereto affixed my signature in presence of two witnesses.

FRANK KAVANAUGH.

Witnesses:

JAMES ROBERT CADE,  
JOHN DIERKEN.